

July 2, 1940.

I. J. NOVAK

2,206,042

WALLBOARD

Filed Dec. 8, 1937

*Fig. 1.*



*Fig. 2.*



*Fig. 3.*



Inventor:  
Izadore J. Novak,  
By: See J. Gary  
Attorney.

## UNITED STATES PATENT OFFICE

2,206,042

## WALLBOARD

Izador J. Novak, Trumbull, Conn., assignor to  
 Raybestos-Manhattan, Inc., Bridgeport, Conn.,  
 a corporation of New Jersey

Application December 8, 1937, Serial No. 178,681

7 Claims. (Cl. 154—2)

This invention relates to improvements in wallboard or plasterboard construction, and particularly to a composite structure of gypsum or plaster and a liner therefor.

5 The object of this invention is to form a liner for gypsum or plasterboard which will readily absorb the moisture or water from the gypsum or plaster and form an adherent and tenacious bond therewith.

10 Another object pertains to the formation of a liner board to which gypsum or plaster may be readily applied and which will readily bond therewith to form a structure which may be readily handled, will not be fragile, which will not be too thick or too bulky, and which may be readily and quickly set up in use without necessity for additional processing.

15 Other objects and advantages will be apparent from consideration of the following specification and description of the drawing, wherein,

20 Fig. 1 is a perspective view of a fragment of wallboard constructed in accordance with an embodiment of my invention, showing an inner layer of gypsum or plaster and outer layers of silicated fibrous material, parts being cut away to illustrate the composition of the composite structure.

25 Fig. 2 is a section through the board shown in Fig. 1.

30 Fig. 3 is a transverse section of a board as it leaves a continuous forming machine.

35 Referring to the drawing, 10 indicates a layer of gypsum or plaster of Paris which has been formed between the layers 11 and 12 of silicated fibre board to form a completed structure which may be readily nailed in place in the form of panels or strips.

40 In Fig. 3 is shown a section of wallboard which has been formed on a continuous forming machine, the bottom paper layer 11 being of greater width than the upper paper layer 12, the edges 13 of the sheet 11 having been bent upwardly to form a trough so as to receive the plastic gypsum and laterally confine it during the setting stage. As 45 the gypsum is poured into the trough formed by the lower sheet, the upper sheet is immediately laid thereon so that the whole may set and bond together. The composite structure or "sandwich" is then passed through suitable roller means while still wet and plastic to form a sheet of uniform thickness and to more firmly consolidate the sheets with the plaster. Then while 50 still wet and before the plaster is set it is passed to a heated dryer to rapidly set the plaster. After the board has been dried, the excess paper

5 at the edges may be suitably trimmed off and the board cut to proper dimensions.

10 The liner board sheets 11 and 12 are formed of fibrous construction by a paper making machine in conventional manner and may be of varying thicknesses consistent with the intended use or desired product. Incorporated with the fibers either by introduction into the pulp in the beater or by the wet web or dry web saturation processes, is sodium silicate, preferably in the proportion of 10 5% relative to the weight of the fibres. The 15 felted fibre sheet may be finished off either by calendering both surfaces or one surface, or both of the surfaces may be left uncalendered, depending upon the desired characteristics of the wallboard; for example, a smooth calendered surface may be used when it is desired to apply directly thereto coating material such as paint or varnish, using a minimum amount of sizing materials, or where it is desired to apply plastic materials to 20 the surface, the sheet may be left uncalendered so as to have a surface wherein the fibres will more readily interlock with plastic materials and form a stronger bond therewith. If it is desired to coat or apply the plaster to the fibrous silicated 25 board after the board has been installed or set in place, a heavier grade of board may be used and gypsum or plaster of Paris in plastic state applied thereto. Or if it is desired to form completed 30 wallboard which will not require a further use of gypsum or plaster of Paris, the plastic material may be sheeted out onto a sheet of silicated fibre board or formed between two thin sheets of 35 silicated fibre board.

40 In addition to the interlocking of the fibres of the fibre board with the plastic material I observe that the silicated fibre board seems to have an affinity for the gypsum or plaster of Paris and there appears to be a chemical reaction at the conjugation of the surface of the silicated fibre board and the gypsum or plaster of Paris so that 45 there is formed between the two an interlocking and adherent bond and while the sodium silicate imparts stiffening characteristics to the structure, it imparts to the fibre board the property of absorbing moisture or water from the plaster of Paris or gypsum. This absorption of water appears to be brought about by hydrolysis of the sodium silicate contained in the fibre board by the moisture of the plastic gypsum to produce an alkaline reaction with the gypsum or plaster of Paris to form a reaction product therewith. While the incorporation of sodium silicate with fibre board permits of the use of a thin board, other alkaline substances may be used in its place, as for ex- 50 55

ample, sodium carbonate, lime, trisodium phosphate, etc., but it has been found that with the use of these other alkaline materials a thicker fibre board is necessary which in many instances is not desirable. However, if alkaline materials are used and the pH value maintained above 8, I have found that this absorption of moisture or water from the plaster by the alkaline substance incorporated with the fibre board will react with the gypsum or plaster of Paris to assist in firmly uniting the fibre board treated with the alkaline substance or sodium silicate, and the layer of plaster.

This results in a firm unitary structure which may be readily handled without crumbling or breaking, may be readily cut up into strips and sizes for use and may be readily shipped or stored. It will also be seen that gypsum or plaster of Paris applied after the fibre board has been installed in construction work or pre-formed in composite wallboard, will readily and quickly dry in a lesser amount of time than is ordinarily required and will set to form a firm bond throughout the whole. Further, by the use of a felted fibrous sheet which may have a smooth calendered surface a wallboard is formed which may be fixed in place and the surface thereof immediately decorated in any suitable surface coating manner, or if it is desired to add additional plaster the surface may be left uncalendered.

In the manufacture of the plaster board "sandwich", it is formed with the silicate treated board that it is immediately wet by the gypsum paste resulting in good adhesion in contradistinction to ordinary chip board which resists water penetration for a much longer time. This rapid penetration of moisture results in more rapid setting of the gypsum, and more rapid drying of the moisture in the dryer end of the continuous forming machine. It was found that the machine could be speeded up 20% to 30% in practice. Further, because of the added stiffness of the board, .015" thickness could be used in place of .019" ordinary chip or news board, resulting in proportional saving. Plaster applied to the outside of the board after installation in a wall adheres satisfactorily without staining.

I claim as my invention:

1. A wallboard comprising a layer of plaster and a felted fibrous liner therefor, the said liner having incorporated therewith an alkaline substance adapted to absorb moisture from the plaster and upon hydrolysis to form a reaction product of said alkaline substance and plaster

and thereby form an adherent bond between said plaster and said liner.

2. The method of making plaster wallboard which comprises forming a felted fibrous liner sheet saturated with sodium silicate, and applying a layer of plastic plaster thereto, a tenacious bond being formed therebetween to interlock the fibres of the said liner to said plaster by the absorption of moisture from the plaster by the sodium silicate and the formation of a reaction product of plaster and sodium silicate upon the resultant hydrolysis thereof. 5

3. The method of making plaster wallboard which comprises forming a felted fibrous liner sheet having incorporated therewith an alkaline body adapted to have a pH value over 8 upon hydrolysis thereof, and applying a plastic layer of plaster thereto, the said alkaline body being adapted to absorb water for hydrolysis thereof from said plastic plaster and to form a reaction product therewith of said alkaline body and said plaster, the said reaction product forming a bonding medium between said liner and said plaster. 15

4. The method of making plaster wallboard which comprises depositing a layer of plastic plaster on a felted fibrous liner sheet comprising sodium silicate, applying a similar liner sheet thereover, the said sheets being adapted by the incorporation therewith of said sodium silicate to absorb water from the said plastic plaster and to react therewith to form a reaction product of sodium silicate and plaster to firmly unite the sheets to said plaster, and subjecting said plastic mass to heat to rapidly set it and to form a firmly bonded unitary board. 25

5. A wallboard comprising an inner core of plaster, and outer plies of felted fibrous material saturated with sodium silicate, and a reaction product of sodium silicate and plaster formed in situ at the conjugation of the respective ply 40 surfaces. 35

6. A wallboard comprising a layer of plaster and a felted fibrous liner therefor, the said liner comprising sodium silicate, and a reaction product of sodium silicate and plaster formed in situ 45 between said layer and said liner.

7. A wallboard comprising a layer of plaster and a felted fibrous liner therefor, and means incorporated with and carried by said liner bonding said plaster thereto, comprising sodium silicate, 50 and a reaction product of sodium silicate and plaster formed in situ on the surface of said layer of plaster.

IZADOR J. NOVAK.